

Nov. 8, 1938.

K. FËHR ET AL  
PROCESS FOR CONVERTING LIQUID PITCH INTO  
A FRAGMENTARY, TRANSPORTABLE FORM  
Filed June 22, 1937

2,136,208



*Inventors:*

Karl Fehr  
Erwin Henemann  
Wilhelm Schneider  
by Mock & Blum  
Attorneys

## UNITED STATES PATENT OFFICE

2,136,208

PROCESS FOR CONVERTING LIQUID PITCH  
INTO A FRAGMENTARY, TRANSPORTABLE  
FORM

Karl Fehr, Erwin Heinemann, and Wilhelm Schneider, Rauxel, Westphalia, Germany, assignors to the firm Bürgerswerke-Aktiengesellschaft, Berlin, Germany

Application June 22, 1937, Serial No. 149,616  
In Germany July 4, 1936

1 Claim. (Cl. 83—81)

This invention relates to a process for converting liquid pitch or liquid pitch-like substances into a fragmentary, transportable form.

In the distillation of coal-tar or other tars after the separation of the volatile constituents a highly heated residue is obtained which is not distillable without being decomposed. Similar residues are obtained in the distillation of numerous other products such as, for instance, petroleum, waxes etc. All these products are called "pitches" such as coal-tar pitch, brown coal-tar pitch, wood-tar pitch, petroleum pitch etc. Their chemical constitutions show considerable differences. On the other hand their physical properties show a great resemblance; they are dark colored, non-volatile, fusible products, insoluble in water and difficultly or only partly soluble in organic solvents. In our present specification and claim the name "pitch" and "pitches" is to be understood as including all the above mentioned products and other similar distillation residues.

It is known that the further working up of pitch or pitch-like substances by chilling or pouring and comminuting the highly heated residue left behind in distillation retorts was hitherto attended with considerable difficulties. On the one hand the objectionable smell and dust accompanying the aforesaid residues constituted considerable disadvantages and on the other hand a considerable expenditure of power and work were necessary in order to convert larger masses of pitch into a fragmentary transportable form.

According to our present invention the chilling or pouring and comminution of the pitch and pitch-like substances are effected in a simple manner without the occurrence of the aforesaid disadvantages of smell and dust and without considerable expenditure of power.

40 In carrying out our invention the still liquid pitch is running off into flowing water and is allowed to solidify and set therein. The solidified pitch whilst still hot is separated in a suitable manner from the water. After the separation from water on further cooling in the air it breaks up into fragments, constituting a transportable and substantially water-free pitch. The water may be used in circulation. The temperature of the flowing water and the relative proportions of water and pitch are so adjusted that the liquid pitch solidifies and the solidified pitch after separation from the water still possesses sufficient latent heat to effect evaporation of the adhering moisture. The operations of chilling, comminut-

ing and transporting the pitch can accordingly be combined into one operation.

## Example 1

Hot liquid pitch at a temperature of 350° C., 5 softening point 150° C., such as is obtained as distillation residue in the manufacture of hard pitch from coal tar is introduced in the form of a thin jet into a channel along which water at 40° C. flows. The pitch quickly sets with a 10 smooth surface without the formation of scum and without water being enclosed in the solidified pitch. For cooling and solidifying 100 kgms. of pitch 2000 kgms. of flowing water at 40° C. may, for instance, be used. The solidified pitch is conveyed by the water stream into a steeply inclined sieve or other suitable device, which is adapted to drain off the water so that the still hot, solidified pitch is to a large extent separated from the water. The temperature of the pitch now 20 amounts to 110° C. and the residual water still adhering to the pitch is evaporated by the latent heat of the pitch, which is then allowed to further cool down in the air. The individual pitch strands then break down on further cooling in the air 25 into fragments, so that the end product constitutes a water-free, fragmentary and transportable pitch. It can thereafter be loaded on to lorries by means of a chute or other known apparatus. 30

## Example 2

The working up of a soft pitch from coal tar having a softening point of 70° C. is carried out essentially in the same manner as described in Example 1. The hot liquid pitch at a temperature of 150° C. is introduced in the form of a thin jet into a channel along which water at 15° C. flows. The pitch quickly sets and is cooled down by the water to about 30° C. The further steps are carried out as described in Example 1. 40

## Example 3

Hot liquid pitch at a temperature of 250° C., softening point 135° C., such as is obtained, as distillation residue, from petroleum runs off into 45 flowing water at 20° C. The pitch sets, its temperature now amounting to 50° C. The further treatment is essentially carried out as described in Example 1.

The accompanying diagrammatic drawing 50 serves to illustrate how the process of this invention may be carried into effect.

The pitch passes out of the container 1, through the outlet 2 into a channel 3 which is fed from the container 5 with flowing water. The water 55

and the pitch leave the channel at the inclined sieve 4. The pitch falls into the conveyer apparatus, whilst the water is withdrawn over an inclined wall 6.

5 What we claim is:

A process for converting liquid pitch into a fragmentary, transportable form by running off the hot liquid pitch in a thin jet into flowing water, mechanically separating the solidified pitch, whilst still hot, from the water, the re-

maining heat evaporating the adhering water from the pitch thus separated by exposing it to air at normal temperature whereby the dissipation of the retained heat in the separated pitch is effective to dry and fragment the same as it cools 5 to normal temperature.

KARL FEHR.

ERWIN HEINEMANN.

WILHELM SCHNEIDER. 10